

# UNITED STATES PATENT OFFICE.

MARY M. HOLDEN, OF NEW YORK, N. Y.

## COMPOSITION FOR BRAKE-BAND LININGS.

1,203,338.

Specification of Letters Patent.

Patented Oct. 31, 1916.

No Drawing.

Application filed April 22, 1916. Serial No. 92,966.

To all whom it may concern:

Be it known that I, MARY M. HOLDEN, a citizen of the United States, residing at the city of New York, in the borough of Brooklyn and State of New York, have invented certain new and useful Improvements in Composition for Brake-Band Linings, of which the following is a full, clear, and exact description.

10 This invention relates to a composition which is adapted for use as a lining for brake bands, brake shoes and the like.

One object of the invention is to provide a composition which, when used as a lining for 15 brake bands, will permit a slight slippage between the member to be braked and the braking member when the brake is first applied and so cause a stoppage of the member to be braked without any sudden shocks 20 or jars.

Another object of the invention is to provide a composition which is softer than the 25 brake drum or the like and yet possesses the requisite coherency between its particles to render unnecessary any reinforcements, such as wire mesh or the like, to hold it together.

Another object is to provide a composition for this purpose which will have a relatively high melting point.

30 Other objects and advantages of my invention will appear from the following description.

The invention consists in a composition of the character described, the essential constituents of which are copper and lead, the lead being in a greater percentage than copper. Preferably, substantially three parts copper and five parts lead are used. Lead is particularly suitable as a component of a 35 brake band lining when combined with a stronger metal for the reason that its properties and characteristics are such that it will permit a slight slippage between the lining and the braking member when the brake band or the like is frictionally applied. A small percentage of phosphorus in the form 45 of phosphor copper may be added to the composition to give it additional toughness and hardness.

50 As is well known, copper in forming an alloy with lead will not take up more than approximately one-half of one per cent. of lead and form with it a true alloy. It is also well known that in forming a lead-copper 55 alloy, lead will not take up more than approximately one-half of one per cent. of

copper. The small quantities of lead and copper which are thus taken up have no material effect upon the characteristics of these two metals and the composition may therefore be regarded as a mechanical mixture of the two. In the mixture, the copper blends or amalgamates with the lead, making the mixture homogeneous throughout. When the composition is therefore cast into bars 60 and utilized as a lining for a brake band, shoe or other form of brake, the lead present in the contacting surface of the lining permits a slight slippage of the brake drum or other member to be braked when the brake 65 band is first applied under a relatively slight pressure. This slippage is not, however, sufficient to prevent a positive braking action from being obtained, since the copper in the composition not only prevents any 70 deformation in the lining due to the flow of lead, but also serves to increase the friction between the lining and drum as the brake band is tightened.

For the preparation of the composition, 80 I have found the following ingredients in the proportions given to be satisfactory: Copper 36 per cent., lead  $62\frac{1}{2}$  per cent., sulfur one half per cent., plaster of Paris one-half per cent., phosphor copper one-half per 85 cent., and with these constituents the composition is prepared as follows: The copper is first melted in a suitable vessel and the lead is then added. Since the melting point of lead is so much lower than the copper, the lead may be added to the molten copper in solid form and will be quickly melted. The lead and copper are then stirred together in order to form as intimate a mixture of the two metals as possible. 90 The copper will then take up a very small percentage of the lead; that is, about one-half of one per cent. and forms with it a copper-lead alloy. The lead also takes up a small quantity of the copper to form 95 with it an alloy, but as before described the formation of these alloys may be disregarded. The sulfur and plaster of Paris or gypsum are then added to purify the metal. The sulfur reduces any metallic oxides of the metals which may be present in small quantities, acting as a reducing agent and converting any of the oxides of lead or copper to metallic copper and lead and giving off  $SO_2$ . The plaster of Paris 100 cleanses the molten mass of metal of other impurities, such as silica, and the like, which 105

forms a thin liquid slag upon the top of the mass of metal within the vessel, which may be skimmed off before casting. After the copper and lead have been purified, phosphorus is added, preferably in the form of phosphor copper which as before stated, tends to toughen the composition. The mixture, before casting, is preferably violently agitated or otherwise treated so as to cause an intimate mixture of the copper and the lead, producing a uniformly blended composition.

It is believed that the homogeneous mixture of the copper and lead is obtained because of the sulfur which is added to the molten mass, since it has been found that without the addition of this sulfur it is very difficult, if not impossible, to obtain an intimate mixture of the lead and copper, which will not separate out before the metal cools.

The composition is in the usual manner cast in bars or in hollow brake shoes so as to form fillers for the same. When cast in bars, it is preferably attached to the brake band or shoe by means of soft copper screws so that the heads of the screws will be worn uniformly with the brake band and will not scratch or injure the face of the brake drum or pulley.

30 I claim:

1. A metallic lining for brake bands and the like containing copper and lead in excess of the copper, the copper content being greater than that which will form a true alloy with the lead.

2. A metallic lining for brake bands and the like containing copper and lead in substantially the proportion of three parts copper to five parts lead.

3. A metallic lining for brake bands and the like containing substantially five parts lead, three parts copper and a small percentage of a phosphorous alloy.

4. The process of preparing a composition for linings for brake bands consisting in first melting a quantity of copper, then adding substantially a larger amount of lead thereto and permitting it to melt, then adding a small percentage of phosphorous alloy, then adding a small percentage of sulfur and plaster of Paris, then skimming the mixture and thoroughly mixing the ingredients as it is allowed to cool.

5. The process of preparing a composition for linings for brake bands, which comprises mixing molten copper, lead and sulfur together, agitating the molten mass and then casting.

6. The process of preparing a composition for linings for brake bands, which comprises mixing molten copper, lead, sulfur, gypsum and phosphorus, then stirring the molten mass, and casting.

In witness whereof, I subscribe my signature, in the presence of two witnesses.

MARY M. HOLDEN.

Witnesses:

JOSEPH HOEHN,  
MAE GROSS.